

## 1

3,684,726

### LUBRICATING GREASE

Alfred Romuald Haak, 2105 Meckelfeld, Mohnweg 11, Germany, and Wolfgang Stichnoth, 15 Muhlenstrasse, 2000 Hamburg 70, Germany  
No Drawing. Filed June 6, 1969, Ser. No. 831,223  
Claims priority, application Germany, June 22, 1968,  
P 17 69 651.4  
Int. Cl. C10m 5/22, 5/16  
U.S. CL. 252—33.2

5 Claims 10

#### ABSTRACT OF THE DISCLOSURE

Lubricating greases comprised of a metal soap and a major amount of mineral oil are improved in their anti-corrosion properties by including in them synergistic mixtures of a barium alkaryl sulfonate wherein the alkaryl group has a molecular weight between 330 and 430 and a naphthenate salt of zinc, lead, lithium or magnesium.

The corrosion of metal parts lubricated by grease in hostile environments is mitigated by including in the grease a synergistic combination of naphthenates and sulphonates.

The present invention relates to lubricating grease. A lubricating grease basically comprises lubricating oil trapped in the interstices of a matrix of soap fibres. The soap is usually a metal salt of a long chain organic acid

| Test number.                                                            | 1   | 2    | 3    | 4    | 5    | 6    | 7    | 8    | 9    | 10   | 11   | 12   | 13   | 14   | 15   |
|-------------------------------------------------------------------------|-----|------|------|------|------|------|------|------|------|------|------|------|------|------|------|
| Grease (90 wt. percent mineral oil plus 10% lithium 12 hydroxystearate) | 100 | 99.5 | 99.0 | 98.0 | 98.0 | 98.0 | 98.0 | 99.5 | 99.0 | 98.0 | 98.5 | 98.0 | 99.0 | 98.0 | 98.0 |
| Lead naphthenate                                                        | 0.5 | 1.0  | 2.0  |      |      |      |      |      |      |      | 1.0  |      | 1.0  |      |      |
| Lithium naphthenate                                                     |     |      | 2.0  |      |      |      |      |      |      |      |      |      |      | 0.5  |      |
| Zinc naphthenate                                                        |     |      |      | 2.0  |      |      |      |      |      |      | 1.0  | 0.5  |      |      | 1.5  |
| Magnesium naphthenate                                                   |     |      |      |      | 2.0  |      |      | 0.5  | 1.0  | 2.0  | 0.5  | 0.5  | 0.5  | 0.5  | 0.5  |
| Barium dinonylnaphthalene sulphonate                                    |     |      |      |      |      | 0.5  | 1.0  | 2.0  | 0.5  | 0.5  | 0.5  | 0.5  | 0.5  | 0.5  | 0.5  |
| Corrosion tests:                                                        |     |      |      |      |      |      |      |      |      |      |      |      |      |      |      |
| DIN 51802 using distilled water                                         | 3   | 2    | 1    | 0    | 0    | 0    | 0    | 0    | 0    | 0    | 0    | 0    | 0    | 0    | 0    |
| DIN 51802 using sea-water according to ASTM D 665                       | 5   | 4    | 3    | 2    | 2    | 1-2  | 4    | 3    | 3    | 2    | 0    | 0    | 1-2  | 0    | 0    |

and among the commonly used soaps are the metal salts of 12-hydroxystearic acid.

Lubricating grease often is employed in situations where moisture can penetrate to the metal parts which are lubricated by the grease, for example, in steam-driven turbines. Greases employed in such situations may contain additives which combat any tendency of the metal parts to become corroded by the moisture. Commonly-used additives are metal salts of naphthenic acid or alternatively metal salts of sulphonic acids. However, these additives are not completely effective in preventing corrosion, and are relatively ineffective where the moisture is associated with inorganic salts, as is the case with seawater.

It has now been discovered, in accordance with the invention, that improved anti-corrosion properties are imparted to a lubricating grease by incorporating in the grease an additive comprising a combination of at least one sulphonate salt and at least one naphthenate salt.

As will be seen from data given below, the combination of sulphonate and naphthenate salts act synergistically to provide corrosion protection of metal parts even in the presence of seawater.

The sulphonate salt is preferably a salt of an alkaline earth metal from Group II(a) of the Mendeleev Periodic table (such as barium, calcium or strontium), but sulphonates of metals in Groups II(b) (such as magnesium and zinc) may also be employed.

The sulphonates may be a petroleum sulphonate or an alkaryl sulphonate. Preferably, the molecular weight of the hydrocarbyl group of the sulphonate is 330 to 430.

The naphthenate may be a salt formed from metals of Groups I to IV of the Mendeleev Periodic table.

A preferred form of grease in accordance with the invention may comprise about 1.5 percent by weight of the naphthenate salt and about 0.5 percent by weight of the sulphonate salt.

The sulphonate salt may be barium dinonylnaphthalene sulphonate, and the metal soap matrix of the grease may be a salt of 12-hydroxystearic acid, such as the lithium salt thereof.

In order to demonstrate the technical advance provided by the invention, a number of tests were performed in accordance with the method of DIN 51802 in which relative rotation is produced between a bearing race and a shaft which are separated by roller bearings, the bearings being lubricated by the grease under test in the presence of a standardized quantity of water. After a standard period of operation, the amount of corrosion is determined.

Each test was performed twice, the first time with distilled water and the second time using a synthetic sea-water formulated in accordance with procedure B of test ASTM D 665.

The amount of corrosion was expressed on an arbitrary scale in which zero corresponds to no corrosion of the surface of the test sample, and 5 designates over 10% of the surface of the test sample corroded. Corrosion of less than 10% of the surface was expressed on a pro rata basis.

The results of the tests are summarised in the following table:

TABLE

An examination of the data in the table shows that in tests 2 to 10, a single additive, either a naphthenate salt or a sulphonate, improved the corrosion protection with respect to the grease alone in test 1, both with distilled water and sea-water according to test DIN 51802.

However, it will be seen that when a combination of one or more naphthenates with the sulphonate is incorporated in the grease, there is a synergistic effect which confers further corrosion protection properties on the grease compared with the amount of protection when only one additive chemical is employed. In the case of tests 12, 14 and 15, there is complete corrosion protection even in the presence of seawater.

In further tests which were carried out, this time in accordance with ASTM D 1743, the basic grease had a corrosion protection of 3 on the scale prescribed in ASTM D 1743. When 2 weight percent of barium dinonylnaphthalene sulphonate was incorporated in the basic grease, the protection as determined by ASTM D 1743 was 2.

Blends were made up of the basic grease with 2% by weight of the naphthenates of lead, zinc and lithium, and tested according to ASTM D 1743. For each blend, the corrosion protection was 2.

It was found that no improvement could be obtained in the corrosion protection by increasing the concentration of the additive in the just described tests.

However, when a grease blend comprising 1 wt. percent of barium dinonylnaphthalene sulphonate and 0.5 wt. percent of zinc naphthenate was tested, the corrosion protection according to ASTM D 1743 was 1, thus demonstrat-

ing the synergistic effect of combining a naphthenate and a sulphonate.

These results serve to confirm the results summarized above in the table.

A grease giving highly satisfactory corrosion performance has been made which comprises about 1.5 weight percent of the naphthenate and about 0.5 weight percent of the sulphonate.

The additives in accordance with the invention do not detract from the lubricating properties of the grease.

We claim:

1. A grease composition comprising mineral lubricating oil thickened with lithium 12-hydroxystearate and containing synergistic corrosion inhibiting proportions of at least one naphthenate salt of a metal selected from the group consisting of lead, zinc, magnesium, and lithium and a barium salt of an alkaryl sulfonic acid wherein the alkaryl group has a molecular weight between 330 and 430.

2. A lubricating grease claimed in claim 1 wherein the naphthenate salt is zinc naphthenate.

3. A lubricating grease as claimed in claim 1 wherein the naphthenate salt is lead naphthenate.

10

15

4. A lubricating grease as claimed in claim 1 wherein the alkaryl sulfonic acid is dinonylnaphthalene sulfonic acid.

5. A lubricating grease according to claim 1 in which the naphthenate forms about 1.5 weight percent and the sulphonate forms about 0.5 weight percent of the grease.

#### References Cited

##### UNITED STATES PATENTS

|           |        |                       |          |
|-----------|--------|-----------------------|----------|
| 2,647,873 | 8/1953 | Matthews et al. ----- | 252—33.2 |
| 3,493,507 | 2/1970 | Haak et al. -----     | 252—33   |

##### OTHER REFERENCES

"Polar-Type Rust Inhibitors" by Baker et al. in Industrial and Engineering Chemistry, vol. 40, No. 12, pp. 2338—2347.

DANIEL E. WYMAN, Primary Examiner

I. VAUGHN, Assistant Examiner

U.S. Cl. X.R.

252—37.7, 389